

1

3,031,402

**LUBRICANT COMPOSITION**

John W. Nelson, Lansing, Ill., assignor to Sinclair Refining Company, New York, N.Y., a corporation of Maine

No Drawing. Filed July 27, 1959, Ser. No. 829,513  
10 Claims. (Cl. 252—51.5)

The present invention relates to oleaginous base lubricants having improved resistance to oxidation. More particularly it relates to lubricants containing certain organic nitrogen compounds, that is a small amount of an amide of an alkyl amine and a di(hydroxy phenyl)-substituted lower aliphatic carboxylic acid.

Mineral oil and synthetic ester lubricants, in the form of greases or free-flowing liquids are called upon to ease friction and prevent damage to machinery operated at temperatures to as high as about 450° F. At these higher temperatures, the internal combustion engine is an ideal oxidizing machine since the motor oil is violently agitated in the presence of air for lengthy periods of time. Greases are subject to similar conditions in their many applications.

Over the range of temperatures developed when employing lubricants, the rate of oil and grease oxidation approximately doubles for each 20° F. rise of temperature. Thus, the oil exposed to aeration at 300° F. may oxidize at a rate about 32 times as great as at 200° F. While well refined motor oils will only oxidize to only a negligible extent at temperatures of the order of 200° F. and lower, oxidation may become quite pronounced at temperatures of 250° F. and higher. In addition, metals act as powerful oxidation catalysts or accelerators; iron, copper and lead being particularly active. The rate of motor oil oxidation may accordingly be increased as much as one hundredfold, at any given temperature, due to exposure to engine metal surfaces, metal particles resulting from normal engine wear, and contamination with combustion chamber blow-by solids and air-borne dust.

All the various types of hydrocarbon constituents of lubricating oils and greases are susceptible to oxidation, if exposed to sufficient air or oxygen and at sufficiently elevated temperatures. Paraffinic hydrocarbons, both straight- and branched-chain, and naphthenic hydrocarbons are readily reactive. Aromatic hydrocarbons, other than some naphthalene and anthracene derivatives, are indicated to be even more susceptible, possibly because of the activating influence of the aromatic ring structure. Synthetic ester lubricants are basically paraffinic in structure differing from hydrocarbon lubricants in many instances by the insertion of ether oxygen atoms in the chain and the partial oxidation of some carbon atoms.

Of even more importance from an engine performance viewpoint are the oxidation end-products formed. Probably one of the first types of oxidation products formed in an oil undergoing oxidation is organic peroxides, which may act as catalysts, causing oxidation of additional components in an oil, or more intensive oxidation of slightly oxidized constituents. Peroxides have also been indicated to be vigorously corrosive to sensitive types of engine bearings. One of the chief end-products of the oxidation of paraffin hydrocarbons is organic acids, ranging from formic and acetic up to high molecular weight fatty acids. Alcohols, aldehydes and ketones also appear to be produced, while more drastic oxidation of paraffin hydrocarbons may yield oxy or hydroxy acid, esters, lactones and complex condensation products of high molecular weight. The acids formed by paraffin oxidation, particularly those of low molecular weight, are vigorously corrosive to copper-lead and cadmium engine bearings. The more complex oxy-acids have been indicated to be

2

a cause of piston ring sticking. Naphthenic hydrocarbons probably oxidize and yield oxy-products in a manner very similar to the paraffins.

The aromatic hydrocarbon constituents of lubricating oils tend to be most readily oxidized, possibly because of the sensitivity of the hydrogen atoms in side chains adjacent to the aromatic ring nucleus, yielding acids and acidic oxy-products of the same general types as the paraffins. Subsequent oxidation of the aromatic ring residue probably results in formation of very complex condensation and polymerization products which tend to be oil insoluble. These types of oxidation products probably constitute the sludges, resins and varnishes which are formed by the oxidation of the more asphaltic or aromatic types of mineral oils. Thus, highly refined, paraffinic oils of high viscosity index tend to become acidic and corrosive to bearings, but do not form excessive oxidation sludges or varnishes in severe engine service, whereas oils of lower V.I. and containing considerable aromatic constituents tend to develop excessive engine sludges and varnishes.

As is well known, commercial lubricating compositions generally contain an oxidation inhibitor. The exact mechanisms by which inhibitors minimize or retard oil oxidation are not known, although it is probable that they function by decomposing organic peroxides as they are formed so that their catalytic effect is nullified. Similarly, inhibitors probably tend to "poison" or counteract metallic catalysts. Inhibitor additives do not eliminate or entirely prevent oxidation of the lubricant when conditions of exposure are severe, and some types of oils are stabilized and improved to a much greater degree by inhibitors than are others. A satisfactorily stable and oxidation resistant oil requires careful refining of the base stocks plus proper selection of the type and concentration of inhibitor most suited to the particular oil.

The art has recognized several types of inhibitors. Elemental sulfur in small amounts can be dissolved in lubricating oils and is quite effective as an oxidation inhibitor. In order to render sulfur less corrosive to copper and still retain its inhibiting effect, it may be reacted with unsaturated fatty oils such as sperm oil or synthetic unsaturated fatty esters of similar general composition. Aromatic and aliphatic sulfides represent another type of compound sometimes utilized as an oxidation and corrosion inhibitor. Relatively simple sulfur-containing aromatics such as dibenzyl sulfide, dixylyl disulfide or dicetyl sulfide are sometimes utilized. More complex compounds of similar type are the alkyl phenol sulfides.

The effectiveness of phosphorous as an oxidation inhibitor in oils has been recognized for many years. Oil-soluble organic compounds of phosphorous such as alkyl and aryl phosphites, e.g., tributyl phosphite and triphenyl phosphite, and aluminum, calcium or barium salts of alkyl phosphoric acids are types of phosphorous compounds which display antioxidant properties. Inhibitors containing both sulfur and phosphorous are usually more effective and efficient in a wider variety of lube oil base stocks than those containing only phosphorous or sulfur, and many of the inhibited motor oils now on the market contain one kind or another of these combination sulfur-phosphorous type additives. One widely used type of sulfur-phosphorous additive is the dithiophosphates, which are prepared by the reaction of phosphorus pentasulfide with alcohols.

Oil soluble organic amines and phenol derivatives such as phenyl- $\alpha$ -naphthyl amine and  $\beta$ -naphthol, have been used for many years as oxidation inhibitors in highly refined turbine oils, lubricating greases and the like. However, compounds of this type display but limited ef-

fectiveness in motor oils under the oxidizing conditions encountered in engines. It has been theorized that these simpler amines and phenols are essentially low temperature inhibitors, and as such are effective only at temperatures below about 200 or 250° F., which is considerably below those to which motor oils are exposed in engines operating at heavy loads. More complex amines and phenol derivatives such as tetramethyl diamino diphenylmethane and alizarin are used to some extent as motor oil inhibitors. However, these compounds are rarely used alone but are applied in conjunction with other types of inhibitors, so that they may be considered more as supplemental additives rather than as primary inhibitors.

It has generally been believed that aliphatic amides have no anti-oxidant properties, but it has now been found that certain carboxylic acid amides are anti-oxidants for oleaginous base lubricating oils. The compositions of this invention incorporate a small amount sufficient to inhibit oxidation, of an acid amide of an alkyl amine in the base oil of lubricating viscosity which is the major portion of the composition. The acid amide is usually present from about 0.005 to 5.0 weight percent of the final lubricant composition, preferably from about 0.05 to 0.5% or 1%.

The novel additive of this invention can be formed by the amidization of a phenol-substituted aliphatic carboxylic acid containing from 4 to 8 carbons in the aliphatic chain containing the carboxyl groups. Especially preferred is 4,4-bis(p-hydroxy phenyl) pentanoic acid,



The phenol group may also be substituted with alkyl or other groups which do not destroy the anti-oxidant effect.

These acids may be prepared by a method described by Yu and Day in the Journal of Organic Chemistry 23, pp. 1004 to 1006 (July 1958). Suitable acids are 3,3-bis(p-hydroxyphenyl) butanoic acid; 3,3-bis(3-methyl-4-hydroxyphenyl) butanoic acid; 3,3-bis(3,5-dimethyl-4-hydroxyphenyl) butanoic acid; 3,3-bis(3-methyl-4-hydroxyphenyl) pentanoic acid and 4,4-bis(3-monochloromethyl-4-hydroxyphenyl) pentanoic acid.

These acids have generally been found to be insoluble in lubricating oil, and the number of the carbon atoms in the amine is usually from about 10 to 50 or more preferably at least 28, to impart oil-compatibility, i.e. soluble, dispersible or miscible properties, to the final product. Primary or secondary amines can be used and I prefer that the amine have at least one alkyl group of at least 16 carbon atoms, e.g. 16 to 24, in a straight chain, most advantageously the amine has two such groups.

Some amines which can be used to supply the amide portion of the novel compounds of the invention are commercial available fatty amines such as: Armeen HT, a hydrogenated tallow amine comprising approximately 71% octadecyl, 24% hexadecyl, 3% octadecenyl and 2% tetradecylamines; Armeen HTD (distilled Armeen HT); Armeen O, a mixture of 85% oleyl, 6% linoleyl, 5% hexadecyl, 4% tetradecyl and 1% stearylamines; Armeen OD (distilled Armeen O); Armeen 18D, distilled octadecylamine; Armeen C, a mostly C<sub>12</sub> amine derived from cocoanut; Armeen CD (distilled Armeen C); Alamine H26D, another distilled tallow amine; Primene 81R, a mixture of branched-chain amines containing 12 to 14 carbon atoms; and Primene JMT, a mixture of branched chain primary amines containing 18 to 21 carbon atoms. Secondary amines useable in this invention include those corresponding to the named primary amines, e.g. dioctydecyl amine, dihexyldecyl amine, dioleylamine, etc. Aliphatic primary diamines, such as those commercially available in the "Duomeen" series which have the requisite

5 carbon content are also suitable materials for use in this invention. For example, Duomeen T, a hydrogenated reaction product of tallow amine and acrylonitrile having a 32 to 50 iodine value and the structure



where R is an alkyl group of 16 to 18 carbon atoms obtained from tallow, may be used.

10 The amides may be used in mineral oil liquid lubricants, mineral oil based greases, synthetic oils and synthetic oil based greases. The additive is prepared by heating and stirring equimolecular quantities of the acid and appropriate amine with sufficient water entraining agent, such as xylene, to obtain a temperature of about 150 to 200° C. 15 for say from about 10 to 25 hours. Boric acid may be used to increase the speed of the reaction. After the theoretical amount of water is removed, the water entraining agent is removed and the product needs no further purification.

15 The lubricating oil base stock used in the present invention is of lubricating viscosity and can be for instance a solvent extracted or solvent refined oil obtained in accordance with conventional methods of solvent refining lubricating oils. Generally, lubricating oils have viscosities from about 20 to 250 SUS at 210° F. The base oil may be derived from paraffinic, naphthenic, asphaltic or mixed base crudes, and if desired, a blend of solvent-treated Mid-Continent neutral and Mid-Continent bright stocks may be employed. A particularly suitable base 20 oil used in the preparation of the composition may be described as a liquid mineral oil fraction having a viscosity index of about 100.

25 Grease compositions may be prepared by the incorporation or formation in the oleaginous base of grease-thickening fatty acid soaps of metals such as the alkaline metals of group I and II of the periodic table. The soap content of the grease is generally about 2-25%. Although the use of high viscosity oils (above 100 SUS at 100° F.) gives harder greases, the use of a low viscosity non-naphthenic 100% solvent refined neutral Mid-Continent base lubricating oil provides a grease having better low temperature pumpability. The soaps are usually the alkali metal or alkaline earth metal, e.g. lithium, barium, calcium, etc.; salts of natural or synthetic long-chain carboxylic acids, such as stearic, hydroxy stearic or lauric acids, say of 12 to 20 carbon atoms.

30 Greases which comprise about 2-25% of the above-mentioned soaps in a synthetic oleaginous base may also be given resistance to oxidation by the use of the phenol-substituted aliphatic acid amide of an N-alkyl amine of this invention. One type of synthetic oleaginous base used is the ester of synthetic oils of lubricating viscosity which consist essentially of carbon, hydrogen and oxygen. Various of these lubricating materials have been described 35 in the literature and generally their viscosity ranges from the light to heavy oils, e.g. about 50 SUS at 100° F. to 250 SUS at 210° F. and preferably 30 to 150 SUS at 210° F. These esters are of improved thermal stability, low acid number, and high flash and fire points. These complex esters, diesters, monoesters and polyesters may be used alone or to achieve the most desirable viscosity 40 characteristics, complex esters, diesters and polyesters may be blended with each other or with naturally-occurring esters like castor oil to produce lubricating compositions 45 of wide viscosity ranges which can be "tailor-made" to meet various specifications. This blending is performed, for example, by stirring together a quantity of diester and complex ester at an elevated temperature, altering the proportions of each component until the desired viscosity 50 is reached.

55 These esters are prepared fundamentally by the action of acids on alcohols. The mere mixture of an alcohol and acid at the proper temperature will react to produce an equilibrium mixture which includes the monoester. 60 The same is true for the reactions of organic dibasic acids

and glycols to produce synthetic lubricant polyester bright stock. The diesters are frequently of the type alcohol-dicarboxylic acid-alcohol, while complex esters are generally of the type X—Y—Z—Y—X in which X represents a monoalcohol residue, Y represents a dicarboxylic acid residue and Z represents a glycol residue and the linkages are ester linkages. These esters have been found to be especially adaptable to the conditions to which turbine engines are exposed, since they can be formulated to give a desirable combination of high flash point, low pour point, and high viscosity at elevated temperature, and need contain no additives which might leave a residue upon volatilization. In addition, many complex esters have shown good stability to shear. Greases which use these esters as the oleaginous base also have most of these characteristics.

Suitable mono- and dicarboxylic acids used to make synthetic ester lubricant bases can be branched or straight chain and saturated or unsaturated and they frequently contain from about 2 to 12 carbon atoms. The alcohols usually contain from about 4 to 12 carbon atoms. In general, the useful glycols include the aliphatic mono-glycols of 4 to 20 or 30 carbon atoms, preferably 4 to 12.

Materials normally incorporated in lubricating oils and greases to impart special characteristics can be added to the composition of this invention. These include corrosion inhibitors, extreme pressure agents, anti-wear agents, etc. The amount of additives included in the composition usually ranges from about 0.01 weight percent up to about 10 weight percent, and in general they can be employed in any amounts desired so long as the composition is not unduly deleteriously affected.

The following example is to be considered illustrative. To a 3-liter round bottom 4-necked flask equipped with a thermometer, motor driven stirrer, reflux condenser, water trap and heating mantle, were charged 214 g. (0.75 mole) 4,4-bis (p-hydroxy phenyl) pentanoic acid, 400 g. (0.75 mole) dioctadecyl amine from hydrogenated tallow and 180 g. of xylene. The mixture was heated and stirred for 14 hours, removing the xylene meanwhile to raise the flask temperature to 200° C. A total of 16.5 cc. of water was obtained. The remainder of the xylene was then removed by heating the product to 225° C. while blowing it with nitrogen. The product weighed 580 g. and represented a 97% yield.

Blends of various proportions of the N-alkyl 4,4-bis(p-hydroxy phenyl) pentamides were made with liquid mineral oil fractions. Table I reports the results of tests made upon some of these blends containing a refined mineral lubricating oil fraction having a viscosity of 537 SUS at 100° F.; 5.44% carbonated, basic barium mahogany sulfonate (15 to 20% concentrate in mineral oil) which gives a barium content of 0.37% to the finished lubricant, 1.8% di-2-methylamyl zinc dithiophosphate diester (50% concentrate in mineral oil) and 0.005% of silicon antifoam agent.

TABLE I  
Railroad Oxidation Test

| Run No. | Sample                                                     | Amide Conc., Percent in Oil | Percent Vis. Rise | Cat. Wt. chg. (mg.) | Acid No. | Pentane Insolubles | Initial pH |
|---------|------------------------------------------------------------|-----------------------------|-------------------|---------------------|----------|--------------------|------------|
| 1.....  | Mineral Oil containing sulfonate and other additives plus— | .....                       | 86.5              | -2.3                | 4.9      | 1.4                | 1.6        |
| 2.....  | N-dioctadecyl 4,4-Bis(p-hydroxy phenyl) pentamide plus—    | 0.5                         | 18.4              | -4.8                | 4.2      | 0.02               | 1.7        |
| 3.....  | N-dioctadecyl 4,4-Bis(p-hydroxy phenyl) pentamide plus—    | 0.1                         | 21.6              | -2.9                | 4.5      | 0.02               | 1.6        |
| 4.....  | N-octadecyl 4,4-Bis(p-hydroxy phenyl) pentamide plus—      | 0.3                         | 23                | -2.8                | 4.5      | 0.02               | 1.8        |
| 5.....  | N-octadecyl 4,4-Bis(p-hydroxy phenyl) pentamide            | 0.6                         | 22                | -4.3                | 4.5      | 0.03               | 1.6        |

The test was the standard Railroad Oxidation test. The test consists essentially of placing 300 ml. portion of a blend in a beaker which contains a weighed amount of

a steel-backed copper-lead catalyst, and oxygen is bubbled into the liquid at a rate of 5 liters per hour. Pentane insolubles are determined by centrifuging the fluid upon completion of the test. A test was also run on a portion of the mineral oil blend containing the additives other than the amide inhibitor to show the anti-oxidant characteristics of the amides of this invention.

The alkaline earth metal sulfonate detergents that may be used, if desired, in my invention are those soluble in the base lubricating oils and obtained for instance, by neutralizing aromatic sulfonic acids with the hydroxides, chlorides, oxides or other inorganic compounds of the alkaline earth metals. Generally, the sulfonate will be sufficient to give the lubricating oil blend an alkaline earth metal content of about 0.2 to 2.0 weight percent. The preferred aromatic sulfonic acids are the oil-soluble mahogany sulfonic acids which can be derived from the treatment of a suitable petroleum oil, such as a liquid petroleum distillate boiling in the range of about 600 to 1000° F., with fuming sulfuric acid or sulfur trioxide, separating the resulting acid sludge from the acid treated oil and recovering the mahogany acids contained in the acid treated oil. The useful mahogany acids generally have a molecular weight of from about 300 to 500 or more, and although their exact chemical structures may vary, it appears that such acids are composed to a large extent of sulfonated aromatic hydrocarbons having either one or two aromatic rings per molecule, possibly with one or more long-chain alkyl groups containing from about 8 to 30 carbon atoms attached to the ring nuclei.

Other suitable aromatic sulfonic acids are the oil-soluble aryl sulfonic acids; such as benzene sulfonic acids and naphthalene sulfonic acids, which include the oil-soluble alkylated aryl sulfonic acids in which the alkyl chain contains from 8 to 18 carbon atoms for instance, dinonyl naphthalene sulfonic acid, and those prepared by reaction of paraffin wax alkyl chains of 20 or more carbons with aromatic nuclei which are then sulfonated

by fuming sulfuric acid, e.g. wax substituted naphthalene. The aromatic oil-soluble sulfonic acids are conveniently employed as a concentrate in the hydrocarbon from which they are derived and are usually present in an approximate 10 to 30 weight percent concentration.

The alkaline earth metal sulfonates of the present invention can be neutral or basic sulfonates. By basic sulfonates is meant those sulfonates in which the alkaline earth metal is present in an amount in excess of that theoretically required to react with the sulfonic acid from which it was made. For instance, there are usually at least about 1.5 equivalents of barium in the sulfonate and in the case of basic calcium sulfonate at least about 1.2 equivalents of calcium. Usually the basic alkaline earth metal sulfonates do not have to have more than 5 equivalents of alkaline earth metal. Also suitable are the oil-

soluble carbonated neutral or basic alkaline earth metal sulfonates.

75 The zinc dithiophosphate anti-oxidants which may, if

desired, be incorporated in the lubricating compositions of my invention are the oil-soluble zinc salts derived from various diester dithiophosphoric acids conventionally prepared by reacting a sulfide of phosphorus, such as phosphorous pentasulfide with an alcohol, phenol or mercaptan. The organic portion in the acid diesters may be an aryl, alkyl, aralkyl or cycloalkyl group which contains from about 4 to 20 carbon atoms, preferably 6 to 14 carbons, and may, if desired, be further substituted. Suitable alcohols which may be employed in preparing the acid esters include primary and secondary alcohols such as 2-methylamyl alcohol, 4-methylpentanol-2, 2-methylpentanol-1, 2-ethylhexanol, diisopropyl carbinol, cyclohexanol, butanol-1 and octadecanol-1, or mixtures of high and low molecular weight alcohols. Other hydroxyl-containing materials which can be reacted with phosphorus sulfide include phenols and alkylated phenols such as dioctylphenol, tri-isobutylphenol and the like. More specifically, the preferred compounds of this group include the zinc salts of dialkyl dithiophosphates such as dihexyl dithiophosphate, diheptyl dithiophosphate, di-lauryl dithiophosphate, di-2-methylamyl dithiophosphate, di-2-ethylhexyl dithiophosphate, and the like.

Particularly suitable zinc dithiophosphates which can be employed are the zinc salts obtained from a mixed dithiophosphate prepared by reacting 2-methylamyl alcohol or a technical mixture of C<sub>7</sub> secondary and C<sub>6</sub> primary alcohols, mainly the former, with phosphorus pentasulfide. The zinc dithiophosphate is employed in my improved lubricating composition in a minor amount sufficient to inhibit oxidation and bearing corrosion and, in most instances, the amount used provides about 0.03 to 0.2 percent by weight of phosphorus on the basis of the lubricating oil in which it is incorporated.

I claim:

1. An oleaginous lubricant composition consisting essentially of a base oil of lubricating viscosity and an amount sufficient to give improved anti-oxidant properties to the composition of an oil-compatible, N-alkyl, bis(hydroxy phenyl) carboxylic acid amide, wherein the carboxylic acid radical is in an aliphatic chain of 4-8 carbon atoms.
2. The lubricant composition of claim 1 in which the base oil is a mineral oil of lubricating viscosity.
3. The lubricant composition of claim 1 where the N-alkyl has two alkyl groups each of which has 16 to 24 carbon atoms.
4. The lubricant composition of claim 1 in which the N-alkyl group contains about 10 to 50 carbon atoms.
- 15 5. The lubricant composition of claim 2 wherein the amide is present in a range of about 0.05 to 1% of the lubricant composition.
6. The lubricant composition of claim 2 in which the N-alkyl group contains about 10 to 50 carbon atoms.
- 20 7. The lubricant composition of claim 3 where the carboxylic acid is 4,4-bis(p-hydroxyphenyl) pentanoic acid.
8. The lubricant composition of claim 4 in which the N-alkyl group contains 28 to 50 carbon atoms.
- 25 9. The lubricant composition of claim 5 in which the N-alkyl group contains about 10 to 50 carbon atoms.
10. The lubricant composition of claim 7 where the N-alkyl is N-dioctadecyl.

References Cited in the file of this patent

Johnson's Di-Phenolic Acid 4,4 Bis (4-Hydroxyphenyl) Pentanoic Acid, pub. February 1959, by S. C. Johnson and Son, Racine, Wisconsin, pages 6 and 24-26.